

Sept. 2, 1952

C. E. SAUNDERS ET AL

2,609,343

OXIDATION INHIBITOR FOR LUBRICATING OILS

Filed July 12, 1948

DYNAMIC OXIDATION TESTS

| SAMPLE                     | TEMP. <sup>°</sup> C | INHIBITORS            | VISCOSITY IN CENTISTOKES<br>AT 100 <sup>°</sup> F |       | NEUTRALIZATION NO. | VOLATILE<br>ACID NO. |
|----------------------------|----------------------|-----------------------|---------------------------------------------------|-------|--------------------|----------------------|
|                            |                      |                       | BEFORE                                            | AFTER |                    |                      |
| DI (2-ETHYLHEXYL) SEBACATE | 130                  | NONE                  | 12.7                                              | 38.0  | 0.02               | 42.2                 |
| DI (2-ETHYLHEXYL) SEBACATE | 130                  | 0.2% PHENOTHIAZINE    | 12.8                                              | 12.9  | 0.02               | 0.03                 |
| DI (2 ETHYLHEXYL) SEBACATE | 150                  | NONE                  | 12.7                                              | SOLID | 0.02               | 80.0                 |
| DI (2-ETHYLHEXYL) SEBACATE | 150                  | 0.2% PHENOTHIAZINE    | 12.8                                              | 12.9  | 0.03               | 0.10                 |
| TETRADECYL SEBACATE        | 130                  | NONE                  | 43.5                                              | 336.  | 0.02               | 77.5                 |
| TETRADECYL SEBACATE        | 130                  | 0.2% PHENOTHIAZINE    | 43.6                                              | 44.0  | 0.03               | 0.04                 |
| TETRADECYL SEBACATE        | 150                  | NONE                  | 43.5                                              | 510.  | 0.03               | 116.2                |
| TETRADECYL SEBACATE        | 150                  | 0.2% PHENOTHIAZINE    | 43.6                                              | 44.1  | 0.03               | 0.08                 |
| TETRADECYL SEBACATE        | 150                  | 0.22% PHENOSELENAZINE | 43.7                                              | 44.8  | 0.03               | 0.08                 |
| TETRADECYL SEBACATE        | 150                  | 0.2% PHENOTELLURAZINE | 43.7                                              | 44.8  | 0.03               | 0.10                 |
| UNDECYL ADIPATE            | 150                  | NONE                  | 16.8                                              | SOLID | 0.02               | 85.0                 |
| UNDECYL ADIPATE            | 150                  | 0.2% PHENOTHIAZINE    | 16.8                                              | 17.9  | 0.03               | 0.11                 |

INVENTORS

CHARLES E. SAUNDERS  
CHARLES M. MURPHY JR.

BY

*Mc Hayes*

ATTORNEY

## UNITED STATES PATENT OFFICE

2,609,343

## OXIDATION INHIBITOR FOR LUBRICATING OILS

Charles E. Saunders and Charles M. Murphy, Jr.,  
Washington, D. C.

Application July 12, 1948, Serial No. 38,196

5 Claims. (Cl. 252—46.3)

(Granted under the act of March 3, 1883, as  
amended April 30, 1928; 370 O. G. 757)

1

This invention relates to oxidation inhibitor additives used with lubricating oils. It relates particularly to such additives used with the relatively new synthetic diester type of lubricating oils.

The prior art of inhibitor additives for lubricants is extensive and includes other types of inhibitors besides those directed specifically toward the protection of the lubricant itself from oxidation, with which the present invention is concerned.

There are many aspects to the problem of lubricant oxidation. For example, considerable variation is found in the products formed upon oxidation of different lubricants, and their effect on different types of lubricated systems. Thus, it is not surprising that a very large number of oxidation-inhibitor additives have been suggested and are in use. These additives fall largely into general groups consisting of aromatic phenolic compounds, aromatic amines, organic sulfur compounds and organometallic compounds.

Most additives were developed for and are now used in (natural occurring) petroleum type oils which have been refined by solvent-treating processes. It is well established that petroleum oils in their natural state contain certain natural oxidation-inhibitors, and that unfortunately these are partially removed by refining operations, particularly solvent-treating processes. However, it is also known that ordinary solvent-refining does not entirely remove these natural inhibitors, and their presence even in small amounts, distinguishes the petroleum oils from the new synthetic oils. And as would be expected, the synthetic oils, though superior in many properties, are definitely inferior to petroleum oils with respect to stability toward oxidation.

It is the general object of this invention to provide a lubricating oil having a high resistance to oxidation.

Another object is to provide such an oil in which the oxidation-inhibitor additive is an inexpensive and readily available chemical compound.

It is the particular object of the invention to provide an oil having the superior lubricant properties characteristic of the synthetic diester oils, and thoroughly inhibited with respect to oxidation deterioration.

In the present invention a highly oxidation resistant lubricating oil is made by the addition of a component of the type:



where X is an element selected from the group, sulfur, selenium and tellurium, and R is either hydrogen or an alkyl radical, or hydrogen in some positions and one or more alkyl radicals in others. The terms commonly used in the art to designate these compounds are "phenothiazine," "phenoselenazine" and phenotellurazine," according to the appropriate specific designation of X. The configuration shown is of the para-type, the hetero-atoms being in the para-(1, 4) relationship to each other.

The invention includes the meta- and ortho- configurations also, typical structures of which are:



The symbols R and X have the same meanings as above.

The accompanying data are presented to illustrate the effectiveness of the inhibitors in several species of diester oils. The data represent results of two types of experiments, viz, laboratory tests and engine runs.

The results of the laboratory dynamic oxidation tests are given in the accompanying data sheet. The test comprises aerating a 25 gram sample with 20 ml. of air per minute for 168 hours in the presence of copper, steel and aluminum specimens. In these tests several different types of oils in one or more viscosity grades were employed for investigation of the effect of the inhibitor. The criteria for the degrees of oxidation occurring in these tests are changes in viscosity and neutralization number, and volatile acid number. Neutralization number, as used in this specification is defined in A. S. T. M. designation: D188-27T. Volatile acid number is a test devised by ourselves whereby the atmosphere of the oxidation cell is continuously conducted through a standard solution of KOH during the run and the extent of neutralization of said solution is determined at the end of the run by back-titration. The results are reported on the same basis as that of neutralization number, viz per gram of oil. We find that the beginning of formation of volatile acids frequently corresponds closely with the end of the induction period for oxidation.

The importance of carrying out tests in the presence of metallic specimens is greater than is immediately apparent. This is because the products formed by action of the oxidation produced acids upon metals may actually catalyze

further oxidation of the lubricant. Thus, some additives which are effective inhibitors of oxidation (as measured by oxygen absorption, e. g.) when tested in glass, are complete failures when tested in metals. As is seen from both the laboratory data and the engine test runs, the lubricants embodying the present invention are very effective in inhibiting oxidation in all its aspects.

Given below are the results of long-run engine tests on two oils, with and without the presence of a small quantity of inhibitor. The tests were made with a 2½ horsepower Onan 10-LS gasoline engine operating under a full load at 1800 R. P. M. Samples were taken before the run and after various periods of time.

The table immediately below shows the effect on oxidation, as measured by neutralization number, of 0.2% phenothiazine added to the diester oil, di-[1-2(2-methylpropyl)-4-ethyloctyl] sebacate. In this specification we conveniently refer to this compound as "tetradecyl sebacate."

| Hours Run | Neutralization Number |             |
|-----------|-----------------------|-------------|
|           | inhibited             | uninhibited |
| 0         | nil                   | 0.01        |
| 94        |                       | 3.6         |
| 96        | 0.08                  |             |
| 164       |                       | 7.6         |
| 180       | 0.12                  |             |
| 286       |                       | 10.1        |
| 300       | 0.16                  |             |
| 500       | 0.30                  |             |

The crankcase temperature was approximately 150° F. The oil capacity of the engine was 2½ quarts and the oil consumption was about 2 ml./hr. for the inhibited oil and about 4 ml./hr. for the uninhibited. After 286 hours, the engine running with the uninhibited oil stopped due to the extremely bad condition of the lubricant. The piston rings and pin were stuck. The interior parts of the engine were all badly varnished. With the inhibited oil the engine was still running after 500 hours and the parts were in good condition. The viscosity of both oils was substantially unchanged during the tests.

The following table shows the effect of the inhibitor with di-(2-ethylhexyl) sebacate, another diester oil. The test conditions were similar to those above and oxidation was measured on the basis of neutralization number and precipitation number. This latter test determines the quantity of naphtha-insoluble material present after oxidation and is described in A. S. T. M. designation: D91-40.

| Hours Run | Neutralization Number |             | Precipitation Number |             |
|-----------|-----------------------|-------------|----------------------|-------------|
|           | inhibited             | uninhibited | inhibited            | uninhibited |
| 0         | 0.01                  | 0.03        | nil                  | nil         |
| 49        |                       | 0.98        |                      | 0.07        |
| 96        |                       | 1.18        |                      | 0.10        |
| 98        | 0.39                  |             | 0.08                 |             |
| 190       |                       | 1.77        |                      | 0.12        |
| 300       | 0.56                  | 2.82        | 0.13                 | 0.17        |

The crankcase temperature was about 145° F. The oil consumption was about 9 ml./hr. for the inhibited oil and about 11 ml./hr. for the uninhibited oil. In this case both engines were run-

ning after 300 hours, but the exhaust valve of that running on the uninhibited oil was sticking and the piston pin was tight. The engine and lubricant, in the inhibited oil test were both in good condition after 300 hours.

A further example of alkyl esters of organic dicarboxylic acids is undecyl adipate.

The foregoing examples are intended to be illustrative only and not limitative except as defined by the herewith appended claims.

The invention described herein may be manufactured and used by or for the Government of the United States of America for governmental purposes without the payment of any royalties thereon or therefor.

What is claimed is:

1. A composition of matter comprising an alkyl diester of an organic dicarboxylic acid and an oxidation-inhibiting amount of a compound selected from the group consisting of phenothiazine, phenoselenazine, and phenotellurazine.

2. A composition of matter comprising an alkyl diester of an organic dicarboxylic acid and an oxidation-inhibiting amount of a compound having the general formula:



where X is an element selected from the group consisting of sulfur, selenium or tellurium, and R represents a member selected from the group consisting of hydrogen and alkyl radicals.

3. A composition of matter comprising the diester oil, tetradecyl sebacate, and an oxidation-inhibiting amount of a compound selected from the group consisting of phenothiazine, phenoselenazine and phenotellurazine.

4. A composition of matter comprising the diester oil, di(2-ethylhexyl) sebacate, and an oxidation-inhibiting amount of a compound selected from the group consisting of phenothiazine, phenoselenazine and phenotellurazine.

5. A composition of matter comprising the diester oil, undecyl adipate, and an oxidation-inhibiting amount of a compound selected from the group consisting of phenothiazine, phenoselenazine and phenotellurazine.

CHARLES E. SAUNDERS.  
CHARLES M. MURPHY, JR.

#### REFERENCES CITED

The following references are of record in the file of this patent:

#### UNITED STATES PATENTS

| Number    | Name     | Date          |
|-----------|----------|---------------|
| 2,190,648 | Cantrell | Feb. 20, 1940 |
| 2,220,723 | Lewis    | Nov. 5, 1940  |
| 2,417,281 | Wasson   | Mar. 11, 1947 |
| 2,466,647 | Stern    | Apr. 5, 1949  |

#### OTHER REFERENCES

"Symposium on Synthetic Lubricants, Amer. Soc. for Testing Materials," Special Tech. Pub. No. 77, June 16-20, 1947, pp. 21 and 22.